

## UNITED STATES PATENT OFFICE

2,576,722

CHLORO-ANACARDIC POLYMERS AND  
METHODS OF MAKING THE SAME

Emil E. Novotny, Prospectville, and George K. Vogelsang, Cheltenham, Pa., assignors to The Borden Company, New York, N. Y., a corporation of New Jersey

No Drawing. Application June 16, 1949.  
Serial No. 99,576

9 Claims. (Cl. 260—46)

1

This invention relates to chloro-anacardic polymers and to methods for making the same. The present application is a continuation in part of application Serial No. 486,432, filed May 10, 1943 (now abandoned). Said application is a continuation in part of application Serial No. 227,528, filed August 30, 1938 (now abandoned), which is in turn a continuation in part of application Serial No. 188,796, filed February 4, 1938. Said last mentioned application matured into Patent No. 2,306,077 on December 22, 1942.

By way of introduction, it may be stated that when chlorinating anacardic material according to the teachings of the above identified patent and patent applications, particularly when the chlorination is carried out at elevated temperatures in the absence of a diluent or modifying agent, a small but nevertheless noticeable amount of condensation-polymerization occurs during the process of chlorination. The condensation-polymerization, which may occur during the process of chlorination, is generally not such as to appreciably alter the character of the ultimate chlorination product which is essentially monomeric in character. Nor is it possible to substantially increase the amount of condensation-polymerization that can occur during the process of chlorination because as the condensation-polymerization progresses the viscosity of the mass soon reaches a point which renders it difficult, if not impossible, to introduce further desirable amounts of chlorine. If a solvent or diluent is used for the purpose of lowering the viscosity, the chlorination proceeds further, but the reaction of condensation-polymerization is slowed down to a negligible degree. It will thus be seen that in the process of chlorination there are self-limiting factors restricting the amount of condensation-polymerization to a low value.

Applicants have now found it possible to obtain a degree of condensation-polymerization, far beyond the maximum normally obtainable during the process of chlorination per se. Furthermore, they have found that the degree of condensation-polymerization can readily be controlled from a low value, which while "low" is nonetheless significantly greater than the maximum obtained during the process of chlorination, to extremely high values. Inasmuch as the process of condensation-polymerization entails a building up of the molecular weight of the material, the mean molecular weight of the product can be conveniently cited as a criterion of the degree of condensation-polymerization.

Briefly stated, the method of the invention consists in subjecting substantially monomeric

chlorinated anacardic material having a chlorine content of at least 10% on the weight of the anacardic material to a heat treatment with or without one or more co-reactants until the mean molecular weight has at least doubled. The chloro-anacardic material is referred to as being "substantially monomeric," because whatever incidental condensation-polymerization, if any, that may have occurred during the process of chlorination is too insignificant to materially alter the character of the chloro-anacardic material, which still has all the attributes associated with monomeric anacardic material.

The starting materials for practicing the present invention are the substantially monomeric chlorinated anacardic materials disclosed in Patent No. 2,306,077 above mentioned and in application Serial No. 458,950 filed September 19, 1942 (now abandoned), the primary object of the invention being to increase greatly the number of useful derivatives of anacardic materials, and to extend their field of utility.

Another very important object is to provide a large number of compounds and compositions having characteristic and unique properties, which render them particularly suitable for many special uses such as synthetic resins and rubbers, plasticizers, co-reactants, etc.

Other objects of importance will appear or will be pointed out as the description proceeds.

The substantially monomeric chlorinated anacardic starting materials may be made in various ways. For instance, anacardic material may be subjected to the action of a chlorinating agent under suitably controlled reaction conditions until the anacardic material has taken up between 10% and 30% of chlorine, based upon the weight of the anacardic material. The chlorinating agent may advantageously be gaseous chlorine, in which case the gas is passed into the anacardic material.

A particularly suitable way of making the starting materials is to mix anacardic materials with a non-anacardic material, and to chlorinate the mixture. The non-anacardic material may be a solvent or non-solvent for the anacardic material, and may be either inert to chlorine or reactive therewith. If the non-anacardic material is reactive with chlorine, sufficient chlorinating agent should be utilized to react with all of the non-anacardic material, and to produce a chlorinated anacardic compound of at least 10% chlorine content. The anacardic material should constitute at least 50% of the mixture of anacardic and non-anacardic materials.

In the presently preferred embodiment of the

2

invention, the non-anacardic material is selected from the group consisting of vegetable and animal oils and fats and their fatty acids.

The chlorinated starting materials are subjected to a treatment or processing to raise their molecular weights and intrinsic viscosity. This treatment or processing may involve the use of heat or reaction with any one or more of a wide variety of powerful reactants or a combination of reactants and heat. A permissible variation is first to heat the chlorinated anacardic materials and then to react the heat-treated material with appropriate co-reagents, preferably with heat.

The principal purpose of the heat treatment is to bring about the desired polymerization, condensation or reaction with the other reactants. Other effects are also brought about. For instance, the more readily volatile materials are driven off, and partial dechlorination takes place. The heat also serves to drive off not only the bulk of the free hydrogen chloride that may be present in the original chlorinated anacardic material but also the hydrogen chloride engendered as a result of the reaction.

Reduced pressures may be utilized during certain phases of the treatment. Partial vacuum serves to remove further quantities of volatile acid material as well as water which is engendered during the heat treatment.

Another permissible variation includes the step of introducing live, preferably super-heated, steam either into the body of the mass or upon the surface thereof. The steam apparently has two functions: First, the use of steam distillation results in a more ready and thorough removal of volatiles and odorous ingredients. Secondly, there is definite evidence that the steam or for that matter hot water enters into reaction with the chlorinated anacardic material resulting in a further elimination of hydrogen chloride concomitant either with the introduction of oxygen, e. g., OH groups into the mass undergoing the heat treatment, or in the introduction of double bonds. The latter may or may not directly attribute to the polymerization of the mass. It should be pointed out, however, that this step of subjecting the chlorinated anacardic material under the influence of heat to the action of steam (or hot water) is entirely optional. Tests made upon the final processed products reveal that the differences in physical and chemical properties of materials processed with or without steam are in the nature of degree rather than of kind. However, it appears that the steam treatment is desirable in that it yields products that are somewhat more stable and exhibit less tendency to give off acidic components in the ultimate articles of which they may be substituents.

Another variation consists in subjecting the chloro-anacardic material first to a heat treatment in a kettle with or without the application of reduced pressures and the action of steam, and then to a further heat treatment, which may be at a higher temperature in an oven. If the time-temperature schedule is sufficiently drastic, the normally liquid products gel and eventually set to a spongy, porous, rubbery mass. In this latter instance large quantities of hydrogen chloride are eliminated. In such a baking operation, it has been found that a certain amount of superficial oxidation occurs. Such oxidation is ordinarily not objectionable but it can be greatly minimized, if not altogether eliminated, by carrying out the further heat treatment in the presence of either

superheated steam or an inert gas such as carbon dioxide, nitrogen, de-oxygenated air, etc. The porous, spongy, puffed-up material may be conveniently homogenized upon different rolls to yield a dense, compact material.

The product of the foregoing procedure may be blended with any one or more of a variety of compounding ingredients so as to yield a fairly stable and neutral material, which lends itself very readily to further processing with substances such as butadiene-acrylonitrile rubbers or polyvinyl acetals, e. g., plasticized polyvinyl butyral.

The following examples are illustrative of the process of the present invention:

15

#### Example 1

Chlorinated anacardic material, with a chlorine content of not less than 10 per cent and preferably between 20 and 28 per cent, is heated in an oven as per the following time-temperature schedule: Slowly bring up to 220° F. Hold at this temperature for about one hour, then raise the temperature to 250° F., holding it there for about an hour. Finally raise the temperature to between 300° F. and 350° F. and maintain this latter temperature for a period depending upon whether the finished product is to be a highly viscous liquid, a rubbery soft solid, or a hard coke-like mass. A four hour period at the elevated temperature usually raises the molecular weight to a point at which is produced a highly viscous product just short of the gel point. A heat treatment at the elevated temperature for a period of approximately six to ten hours usually yields a puffed-up spongy soft rubbery mass. It is to be noted that in this particular example no stirring or agitation is employed. This, in a sense, has the disadvantage of yielding a somewhat non-uniform product. However, for many purposes the material after blending on differential rolls (in the instance of the soft solid) yields a product of adequate uniformity.

#### Example 2

Chlorinated anacardic material prepared in accordance with the disclosure of Patent No. 2,306,077 is placed into a glass-lined kettle provided with an agitator and facilities for heating and cooling. The mass is first gently heated, and when the product is liquid enough the agitator is started and kept running. When the temperature attains a value of between 210° F. and 230° F., a very decided quantity of foam is engendered due to the elimination of water and other ready volatiles. In this phase of the operation the amount of heat that can be applied to the mass is strictly limited by the amount of foam that it is permissible to engender, this latter being determined by the free volume of the kettle. The foam, however, soon subsides and from that time on ever increasing amounts of heat can be applied to the reaction mass. It is desirable not to exceed a temperature of 320° F., and if possible, to maintain a temperature no higher than 300° F. The material is conveniently kept at or above 275° F. for a period of about four hours, and the result is a product of substantially higher molecular weight having a viscosity comparable to that of heavy molasses. Such material has utility as a plasticizer for rubber as well as for a wide variety of other purposes. This material is also capable of being thermoset by a wide variety of reagents including hexamethylenetetramine, formaldehyde, reactive keto-aldehyde reaction products, many of the more powerful accelerators for natural rub-

ber, etc. The physical and chemical properties of the ultimate material depend in large measure upon the original or ultimate chlorine content. When it is desired to produce plasticizers, chlorinated anacardic materials with chlorine contents of between 15 and 20 per cent are preferably used. When it is desired to produce materials which, as is more fully explained in a further example, are to be used as rubber extenders or as binders in conjunction with polyvinyl butyral, chloro-anacardic materials with chlorine contents of between 20 and 30 per cent, e. g. 22 to 26 per cent of chlorine, are preferably used.

*Example 3*

Chlorinated anacardic material prepared in accordance with the disclosure of Patent No. 2,306,077 is placed into a glass lined kettle provided with a stirrer and means for heating. The material is slowly heated. When the mass becomes sufficiently fluid the stirrer is started, and from this time on the mass is continuously stirred. The temperature is gradually raised until the mass foams up. After the foam has subsided the heating is continued until a temperature of 240° F. or higher is attained, at which time vacuum is slowly applied to the kettle. The temperature is either maintained at the previous level or is raised to between 280° F. and 335° F., during the whole of which time the vacuum is maintained. The material is kept under vacuum within the above temperature range for a period of time which depends upon the desired viscosity of whether a soft rubbery product is desired. In the latter instance, the stirrer must be stopped just prior to the gelling. When the reaction of condensation or polymerization has proceeded to the proper point, the vacuum is shut off and the material withdrawn from the kettle. It will be noted that in the instance where the end product is a soft rubbery material, carrying out of the whole of the operation in a kettle has the disadvantage that the kettle must be dismantled in order to remove the product. For this reason, the reaction is preferably carried out in the kettle well short of the point where the mass sets up, and the fluid product is then withdrawn into pans which are placed in an oven. It is a relatively simple matter to remove the rubbery product from such pans. Material processed with the aid of vacuum is quite similar to that processed without vacuum, except that the material is somewhat freer of volatiles and odorous constituents.

The products of the foregoing process have molecular weights which are very much higher than that of the highly viscous products of Examples 1 and 2, indeed the molecular weights are usually so high that they cannot be determined by ordinary methods.

*Example 4*

Chlorinated anacardic material prepared in accordance with the disclosure of Patent No. 2,306,077 is placed into a kettle provided with a stirrer and facilities for heating the mass proper as well as for introducing steam into the mass or blowing the same over the surface. The material is slowly heated until the mass is liquid enough so that agitation may be started. The temperature is raised with continued agitation until the mass foams. After the foaming has subsided, the heating is continued with agitation until a temperature of approximately 240° F. to 335° F. is attained. Then steam, preferably dried

or super heated, is blown over the surface of the mass or bubbled through the mass while maintaining the material within the stated temperature range. The processing is continued until the desired increase in molecular weight has occurred. The fluid mass is then withdrawn from the kettle and may, if desired, be subjected to further processing as described elsewhere. Material subjected to the above steam treatment is quite similar to material processed without the aid of steam, but is freer of objectionable odors and has less tendency to liberate acidic products.

*Example 5*

15 Chlorinated anacardic material prepared in accordance with the disclosure of Patent No. 2,306,077 is placed into a glass lined kettle provided with an agitator and facilities for vacuum and the blowing in of steam either through the 20 mass or on the surface of the material. The material is slowly heated. The agitator is started as soon as possible and kept running throughout the remainder of the operation. The heating is continued until the material foams. After defoaming, the temperature is raised to above 220° F., at 25 which time a greater or lesser vacuum is applied. The vacuum is maintained for a period that may vary from fifteen minutes to a few hours. The vacuum is then discontinued, and in lieu thereof steam is either blown onto the surface of the material or passed through the same. During this steaming operation, it is desirable to maintain temperatures of between 250° F. and 335° F. (preferably 280° F. to 310° F.). When the molecular 30 weight has reached the desired point the material is withdrawn from the kettle. If desired, the product may be subjected to further processing as in an oven. The steaming may advantageously precede the vacuum step.

*Example 6*

The molecular weight of the processed chloro-anacardic material of Examples 2, 3, 4 or 5 may be increased by placing the material into pans 45 which are set into an oven where the material is subjected to a further heat treatment. For most applications, it is desirable to maintain an oven temperature of between 300° F. and 350° F. The material gradually further thickens and then gels. 50 The gel gradually stiffens and concomitantly therewith, particularly if higher temperatures are maintained, the product foams and puffs up. Considerable acrid vapor and fumes are eliminated in this step. The baking operation is continued until the desired degree of reaction has 55 been obtained. If the material is left in the oven long enough, it becomes hard and brittle, in which case it is particularly suitable for use as a filler in the manufacture of frictional elements. If 60 the product is to be used in formulating a rubber or resin mix, the material should be removed from the oven while still soft and rubbery.

*Example 7*

65 Experimentation has disclosed that the more highly condensed and polymerized the product is, i. e. the higher the molecular weight the stronger and more suitable it becomes for use as a rubber extender or as a co-reactant for vinyl derivatives such as polyvinyl butyral or for purposes of co-curing the same with such materials. Such highly polymerized or condensed products, however, because of their high molecular weight, have such high intrinsic viscosity, that they are 70 virtually non-pourable at room temperatures,

This difficulty can be circumvented by adding to the material in the kettle just prior to normal pour time an appropriate quantity of a suitable diluent in the nature of a solvent or plasticizer. Thus one may incorporate a plasticizer such as dioctyl phthalate or dibutoxy-ethyl-phthalate. The use of a quantity of plasticizer equal to the weight of the processed chlorinated anacardic material is typical. For applications where this type of product is desired, it is desirable to process chlor-anacardic material just short of the gel point.

*Example 8*

Chlorinated anacardic material which has had its molecular weight increased until it is in the form of a soft rubbery solid is milled upon differential rolls with appropriate compounding ingredients calculated to impart the elements of neutrality and stability to the same as well as to enhance the processing qualities. The following is a typical formulation:

|                                                                                    | Parts  |
|------------------------------------------------------------------------------------|--------|
| Processed chlorinated anacardic material<br>in the form of a soft rubbery material | 100.00 |
| Zinc oxide                                                                         | 18.38  |
| Magnesium oxide, light calcined                                                    | 6.03   |
| Butadiene-acrylonitrile copolymer rubber                                           | 5.40   |
| Plasticizer                                                                        | 1.32   |
| Cerese Wax (micro-crystalline paraffin<br>wax)                                     | 0.70   |
| Blended waxes                                                                      | 0.40   |
| Phenylethanolamine                                                                 | 0.20   |
| Benzothiasyl disulphide                                                            | 0.09   |
| Phenylbetanaphthylamine                                                            | 0.06   |
| Stearic acid                                                                       | 0.06   |

The above ingredients, when thoroughly mill processed, yield a strong, tough, and highly flexible material which is suitable as a substitute for rubber in certain applications. The product is highly effective as an extender of rubbers of the butadiene-acrylonitrile copolymer type.

As has already been pointed out, the physical and chemical attributes of the final products are in large measure dependent upon the chlorine content of the chlorinated anacardic material as well as upon the type and quantity of other agents that may be contained in the chlorinated material. The following is a typical formulation for a chlorinated anacardic material which is pre-eminently adapted for use as a raw material in the production of the products of the present invention, particularly those designed for use as rubber extenders, polyvinyl acetal extenders, etc.

|                             | Parts |
|-----------------------------|-------|
| Defoamed anacardic material | 60.00 |
| Tetrachlorethane (diluent)  | 4.50  |
| Palm oil fatty acid         | 0.50  |
| Linseed oil fatty acid      | 0.25  |
| Pine oil                    | 0.75  |
| Chlorine                    | 18.75 |

Excellent results are obtained when the chlorination is carried out in a period of between six and eight hours at a temperature of approximately 175° F.

When it is desired to produce a plasticizer, it is recommended that a smaller quantity of chlorine be introduced.

Chlorinated anacardic material, preferably after the molecular weight has been increased by one of the heat treatments above described, may be admixed with material such as lime, zinc oxide, magnesia, etc., to yield compositions which, when heat treated, set up to yield materials simulating

slate. Fillers such as asbestos floats may be incorporated to advantage.

By adding moderate quantities of copper oxide, copper acetate, copper chloride, ferric chloride, chromates, bichromates, etc., to chlorinated anacardic material, preferably after a preliminary heat treatment, it is possible, by subjecting the mixture to adequate temperatures in an oven, to obtain spongy, porous coke-like masses which may be ground up to yield the material between 100 and 300 mesh. The products are preeminently suited for the manufacture of frictional elements, e. g., clutch facings and brake linings. In the above reactions, a substantial amount of "cross-linking" occurs, leading to the formation of very high molecular weight complexes.

The process of the present invention may also be carried out without the use of appreciable heat, provided that very powerful co-reactants are utilized. Thus chloro-anacardic material may be admixed with hexamethylenetetramine, strongly acidic materials, agents which liberate strongly acidic materials, or the very powerful agents belonging to the group consisting of the saturated halogenation products of the aldehydes of the mono hetero atomic five membered rings and their reactive derivatives, and allowed to stand for a period of time. The resultant polymers are essentially of the condensation type. It is to be noted, however, that superior products result from the use of heat as disclosed in the given examples.

The condensation-polymerization products of the present invention have much higher molecular weights than the unprocessed chloro-anacardic materials from which they were derived. The chlorination of anacardic material leads to the production of substantially monomeric chlorination products. Whatever polymerization-condensation may occur during the process of chlorination per se is of negligible import and does not appreciably alter the monomeric character of the material. Experiments have shown that in order that the condensation-polymerization exert an effect sufficiently large so as to enable one to readily distinguish between the original substantially monomeric product and the derived product, the mean molecular weight should be at least double that of the original substantially monomeric material. When the molecular weight of the processed material is double that of the original substantially monomeric chlorinated material, the polymerized material acquires attributes which permit one to readily distinguish the same from the original material. In most technical applications, it is desirable to increase the weight many times over the above that of the original material. Thus, while an original product may have a mean molecular weight in the neighborhood of 600, a thick viscous product short of the rubbery point may possess a mean molecular weight in the neighborhood of between 5,000 and 20,000. The molecular weights of the soft rubbery or the still harder polymers are correspondingly higher.

It is not known for a certainty whether these products are polymerization polymers or condensation polymers. There are definite indications, however, that the mechanism of polymer formation partakes of both types of polymerization. Accordingly, the products of the present invention may be described as chloro-anacardic polymerization-condensation polymers or more briefly as chloro-anacardic polymers. In the interest of clarity and brevity, the polymers of the

present invention are hereinafter referred to as chloro-anacardic polymers.

Chloro-anacardic polymers, if in the form of viscous liquids, gels, or soft rubber products, can be converted into slate-like products by curing them in the presence of a wide variety of agents as typified by lime, zinc oxide, sulphur, paraformaldehyde, hexamethylenetetramine, formalin, as well as the vast majority of the organic accelerators such as are used in the compounding of natural rubber, the saturated halogenation products of the aldehydes of the mono-hetero atomic five membered rings and their reactive derivatives, etc. These products may be used as substitutes for slate blackboards or, if ground up, are useful as fillers in the manufacture of frictional elements.

The soft rubbery polymers are particularly suitable for use as rubber extenders or as compounding ingredients to be used in conjunction with rubber, either natural or synthetic.

The products of the present invention, particularly those processed just short of the gel point (which are conveniently used in admixture with plasticizers for the purpose of imparting a working fluidity to the whole) are preeminently suited for co-vulcanization with polyvinyl acetals, e. g., polyvinyl butyral.

Typewriter platens containing equal parts of natural rubber and one of the foregoing chloro-anacardic rubbery polymers together with the usual compounding ingredients are exceptionally tough, durable, resilient, and are capable of producing a large number of copies. They have a frictionally smooth and velvety surface not subject to rapid hardening.

Many of the chloro-anacardic polymers, particularly those of a soft rubbery nature, are suitable for use as "carriers" for agents which, in and of themselves cannot be conveniently handled. Thus the pungent and acrid saturated halogenation products of the aldehydes of the mono-hetero atomic five membered rings and their reactive derivatives may be readily milled into the soft rubbery chloro-anacardic polymers to yield rubbery products which cannot readily be handled in the conventional manner.

The softer and more fluid polymers prepared according to the present disclosure are very useful as plasticizers for a wide variety of products including natural and synthetic rubbers, the polyvinyl acetals, a wide variety of cellulosic derivatives, phenolic resins, aminoaldehyde resins, furfur-acetone resins, gum accroides resins, resins processed out of dragon's blood, etc.

Many of the chloro-anacardic polymers, possessing as they do an inherent and intrinsic rubbery quality, are preeminently adapted for incorporation into a wide variety of resins, e. g. those of the phenol-aldehyde and amino-aldehyde types, for the purpose of imparting improved flexibility, decreased brittleness, and in general improved machinability. Chloro-anacardic polymers are also ideally adapted for use as fluxing agents, flow aids, and lubricants in the manufacture of molding compositions.

Chloro-anacardic polymers may be reacted with phenols as well as with a wide variety of resins such as the phenol-formaldehyde and phenol-furfural resins to yield resinous compositions possessing new and unique qualities. Such modified resins are of particular value in applications where extensive machining is necessary as well as where high heat resistance and good electrical properties are called for.

The more rubbery polymers can be used by themselves in the manufacture of gaskets and sealing rings as well as other articles previously made of rubber. The more fluid polymers, which 5 partake of the nature of liquid resins rather than of those of plasticizers, are useful as impregnating materials either alone or in conjunction with other resins.

The invention has been described in connection 10 with a number of illustrative embodiments, materials, proportions, conditions and arrangements of operations for carrying out its teachings. It is, therefore, to be understood that the invention is not to be restricted to the foregoing disclosure, 15 and that no limitations are to be imposed which are not required by the language of the appended claims and the state of the prior art. It is further to be understood that the invention is not dependent upon any explanations or theories which have 20 been set forth as descriptive of the actions involved, nor dependent upon the accuracy or soundness of any theoretical statements so advanced.

We claim:

25 1. The method of preparing chloro-anacardic polymers which comprises heating a substantially monomeric chlorinated anacardic material having a chlorine content of between 10% and 30% to a temperature between 240° and 350° F. until 30 the mean molecular weight has increased to at least double that of the original chloro-anacardic material, the said heat being used as the sole agent to effect the polymerization.

2. The method of preparing chloro-anacardic 35 polymers which comprises heating a substantially monomeric chlorinated anacardic material having a chlorine content of between 10% and 30% to a temperature between 240° and 350° F. until the mean molecular weight has increased to at 40 least double that of the original chloro-anacardic material, and the product is substantially free of ready volatiles, the said heat being used as the sole agent to effect the polymerization.

3. A method of preparing chloro-anacardic 45 polymers which comprises subjecting a substantially monomeric chlorinated anacardic material having a chlorine content of between 10% and 30% to the action of heat and steam until the mean molecular weight has increased to at least 50 double that of the original chloro-anacardic material and the product is substantially free of ready volatiles, the said heat being used as the sole agent to effect the polymerization.

4. The method defined in claim 1, the heating 55 step being carried out below atmospheric pressure.

5. The method defined in claim 1, the material being subjected to the action of steam during at least part of the heating step.

6. The method defined in claim 1, the material 60 being subjected to the action of steam during part of the heating step and being maintained below atmospheric pressure during another part of the heating step.

7. The method of preparing chloro-anacardic 65 polymers, which consists in subjecting anacardic material to the action of a chlorinating agent until the anacardic material has taken up from 10% to 30% of chlorine based on the weight of the anacardic material to produce a substantially 70 monomeric chlorinated anacardic material, and after the completion of the chlorination step heating the monomeric chlorinated anacardic material until its mean molecular weight has increased to at least double that of the monomeric 75 chlorinated anacardic material, the said heat

11

being used as the sole agent to effect the polymerization.

8. Chloro-anacardic polymers made by the method defined in claim 1.

9. Chloro-anacardic polymers made by the method defined in claim 3.

EMIL E. NOVOTNY.

GEORGE K. VOGELSANG.

12

## UNITED STATES PATENTS

| Number    | Name           | Date          |
|-----------|----------------|---------------|
| 2,306,077 | Novotny et al. | Dec. 22, 1942 |
| 2,399,735 | Harvey         | May 7, 1946   |

## OTHER REFERENCES

Mattiello: Protective and Decorative Coatings, vol. I, 1941, page 98.

## REFERENCES CITED

10

The following references are of record in the file of this patent: